

# United States Patent Office

2,946,729

Patented July 26, 1960

1

2,946,729

## PRODUCTION OF ELECTROLYTIC ZIRCONIUM

Reginald S. Dean, Hyattsville, Md., assignor to Chicago Development Corporation, Riverdale, Md., a corporation of Delaware

No Drawing. Filed June 9, 1958, Ser. No. 740,568

1 Claim. (Cl. 204—64)

This invention relates to the production of electrolytic zirconium. It has for its aim the production of coarsely crystalline zirconium adherent to an inert conducting cathode from a molten bath of alkalinous metal chloride and lower zirconium chlorides.

In my copending applications, Serial No. 605,232, filed August 20, 1956; Serial No. 638,901, filed February 8, 1957; and Serial No. 647,206, filed March 20, 1957, now abandoned, I have disclosed the formation of coarsely crystalline intergrowths of pure metals of groups IV-B, V-B and VI-B in characteristic form of a thin layer of the metal on the cathode growing into a layer of fine crystals in salt and finally into coarse crystal intergrowths of the metal frangibly attached to said salt layer. The intergrowths constituting 90% or more of the metal adherent to the cathode. I have disclosed that the formation of these intergrowths is due to their crystallization from a supersaturated solution in a melt of alkalinous metal chloride and dissolved therein two chlorides of the metal to be deposited and free alkalinous metal.

The production of titanium in the form described and by the procedure described, has been disclosed in the above copending applications.

The ternary system Zr—Cl—Na differs from the analogous titanium system by the existence of a stable compound ZrCl, which is insoluble in molten alkalinous chloride. This compound forms a layered lattice of semi-metallic character and occurs as small shiny flakes.

The pseudobinary system ZrCl—NaCl divides the ternary system into two composition areas, above the line, the melt is in equilibrium with Zr and so behaves analogously to titanium, below the line, the stable solid phase is ZrCl.

In order to function satisfactorily as an electrolyte, the composition of the single phase liquid must be prevented from changing in composition so as to fall below the pseudobinary line ZrCl—NaCl. This is rendered difficult by reactions not encountered in the case of titanium and other metals of groups IV-B, V-B and VI-B of the periodic system.

These may be listed as follows:



Reaction 1 is a general electrolyte reaction driven from right to left by the volatility of ZrCl<sub>4</sub> and depleting the electrolyte in soluble Zr eventually to the point of uselessness. Reaction 2 occurs at metallic zirconium anode material and also depletes the electrolyte.

The result of these two side reactions is that sooner or later the electrolyte becomes essentially NaCl+ZrCl with a little dissolved Zr<sup>IV</sup>.

There are several ways of combating these side reactions. Reaction 1 is inhibited by conducting the electrolysis under pressure as disclosed in our copending application. I have, however, found it sometimes preferable to drive Reaction 1 from right to left by periodic

2

additions to the electrolyte of a stoichiometric mixture of ZrCl<sub>4</sub> and ZrCl to form ZrCl<sub>2.1-2.4</sub> and sodium according to the reactions



where x is from 2-3.

Reaction 2 gradually degenerated the anode residue into ZrCl and if the electrolyte is maintained by adding ZrCl+ZrCl<sub>4</sub>, this may simply be allowed to continue and the ZrCl recovered periodically and used to add with the ZrCl<sub>4</sub>, which is also recovered from the cooler parts of the apparatus.

15 ZrCl is conveniently made by heating ZrCl<sub>4</sub> and Zr in molten NaCl under pressure for a long period. For purposes of replenishing the electrolyte, the product may be added directly to the cell.

ZrCl can also be made electrolytically by passing a direct current through a cell having a particulate anode of Zr and an electrolyte of alkalinous metal chloride and ZrCl<sub>4</sub>. For this purpose, a low melting electrolyte like SrCl<sub>2</sub> 65%, NaCl 35% is desirable. Several percent of ZrCl<sub>4</sub> can be dissolved in such an electrolyte at 1100° F. The ZrCl<sub>4</sub> is obtained more or less adherent to the cathode in the form of graphitic appearing flakes.

20 From either product containing ZrCl, it may be recovered by dissolving the salt in dilute HCl. The flakes after thorough washing analyze approximately ZrCl.

25 Since other metals of the titanium group including hafnium do not form an analogous compound, the washed flakes contain only zirconium and chlorine. This method may, therefore, be used as a separation from hafnium.

30 It will be recognized that ZrCl can also be made by sodium reaction of ZrCl<sub>4</sub> by long heating of ZrCl<sub>4</sub> under pressure with the stoichiometric requirement of sodium. This reaction goes primarily to metallic Zr and ZrCl<sub>2</sub>, however, after long heating, ZrCl is formed. It is preferable, however, to accomplish this in two stages, reduction to finely divided Zr in the first stage and then reaction with ZrCl<sub>4</sub> by one of the methods above.

35 The flakes of ZrCl have practically important properties. They are semi-conductors, but more importantly, because of their layered structure of alternate metal and non-metal ions, they are condensers of atomic dimensions and show substantially no change of capacity with frequency.

40 As a practical means of operating large refining cells, the maintenance of the electrolyte can be accomplished by having one the bottom of the cell a large reservoir of Zr+ZrCl to which is added periodically ZrCl<sub>4</sub> to provide formation of ZrCl<sub>2.1-2.4</sub> for the electrolyte by the reactions



The anode basket can be eliminated; it is, however, preferable to maintain it and when its contents have too far become ZrCl simply place this in the reservoir at the bottom of the cell and replace it with Zr to be refined.

### Example I

In this example, I take an electrolytic cell having an inert atmosphere, a centrally located steel cathode surrounded with a steel anode basket containing comminuted zirconium scrap. I place sodium chloride in the cell and add a mixture of ZrCl and ZrCl<sub>4</sub> in the proportions necessary to provide an electrolyte containing 4% dissolved Zr as chloride, average valence 2.1. I find that this electrolyte contains 1.2% free sodium as determined by hydrogen evolution in acidified FeCl<sub>3</sub>. I electrolyze at a current density of 200 amps./sq. ft. on the cathode. Anode current density is less than .01 amp./sq. ft. I add

$ZrCl_4 + ZrCl_4$  at regular intervals to maintain the electrolyte.

The anode material analyzed

|                                  | Percent |
|----------------------------------|---------|
| Tin                              | 1.0     |
| Iron                             | 0.3     |
| $O_2$                            | 0.15    |
| Balance substantially zirconium. |         |

The cathode product which was coarse crystal intergrowths formed on the cathode surmounting a zirconium plate and a layer of salt with fine crystals of zirconium distributed therethrough.

After washing with dilute acid, the zirconium crystal intergrowths analyzed

|       | Percent |
|-------|---------|
| Tin   | .0001   |
| Iron  | .002    |
| $O_2$ | .005    |

When melted in an inert atmosphere furnace, the hardness of the zirconium was Vickers 72.

#### Example II

In this example, I proceed as in Example I up to the point of starting the electrolysis. I then add a large amount of comminuted zirconium scrap at the bottom of the cell and I maintain the electrolyte as electrolysis proceeds as in Example I with regular additions of  $ZrCl_4$  only.

The results are identical with Example I.

#### Example III

In this example, I make  $ZrCl$  for carrying out the previous examples by heating 90 grams finely comminuted zirconium, 170 grams  $ZrCl_4$  and 200 grams sodium chloride in a closed vessel at  $850^\circ C$ . for 48 hours. I use the product which is mostly  $ZrCl_4 + NaCl$  to mix with  $ZrCl_4$  and replenish the bath as in Example I.

#### Example IV

In this example, I make  $ZrCl$  from zirconium sponge containing 3% Hf and  $ZrCl_4$  containing 3% of the weight of Zr as Hf by making the sponge an anode in a cell having an inert atmosphere and a steel cathode surrounded by an anode basket containing the zirconium.

The electrolyte is 65%  $SrCl_2$  35%  $NaCl$  containing 2% Zr as  $ZrCl_4$ . The electrolysis is carried on at  $1100^\circ F$ . The current density on the cathode is 400 amperes/sq. ft. There is deposited on the cathode a loosely adhering deposit of flakes. These flakes are washed with dilute HCl and water and analyze 25.2% Cl corresponding approximately to  $ZrCl$ .

The flakes are hafnium free. X-ray studies reveal a layered lattice of Zr and Cl. Measurements of capacity show the flakes to behave as condensers having a capacity independent of frequency.

#### Example V

In this example, I produce the initial electrolyte by heating the materials in the proportion of the following equation in a sealed stainless steel bomb to  $850^\circ C$ . for 48 hours.



This electrolyte when removed from the cooled bomb analyzed

4% soluble zirconium

Average valence, 2.2

Sodium equivalent to 6 cc. hydrogen/gram evolved in 70 acified  $FeCl_3$

The  $ZrCl_4$  pressure of this electrolyte at  $850^\circ C$ . was 75 mm. Hg.

I place this electrolyte in a cell so arranged that the electrolyte is separated from the upper part of the cell by a barrier in a heated zone at  $850^\circ C$ . which has only capillary openings to the top part of the cell which is cool. The top part of the cell is maintained at an argon pressure of 75 mm. to prevent diffusion of  $ZrCl_4$  into the cooler parts of the cell.

I place in the cell a centrally located steel cathode and surrounding it in the electrolyte a steel basket containing the crude comminuted zirconium to be refined.

I pass a direct current through the cell with the basket of crude comminuted zirconium as anode.

The current density on the cathode is 500 amperes/sq. ft. and on the anode material less than 1 ampere/sq. ft. Coarse crystalline zirconium free from  $ZrCl$  is deposited adherent to the cathode.

After washing with dilute HCl the cathode product analyzed:

|       | Percent        |
|-------|----------------|
| Zr    | 99.99+         |
| $O_2$ | .02            |
| Fe    | .001           |
| $N_2$ | .001           |
| Hf    | Less than .004 |

with substantially no other impurities.

The crude zirconium used as anode material analyzed:

|       | Percent |
|-------|---------|
| $O_2$ | 1.2     |
| Fe    | 3       |
| $N_2$ | 0.2     |
| Hf    | 2.8     |

Balance substantially zirconium.

#### Example VI

In this example, I make the electrolyte of Example V by heating in a sealed container  $ZrCl_4$  with Na in the proportions to form  $ZrCl_2$  and  $NaCl$ . This product contains about 22% Zr. To produce the electrolyte, it is added to 4 times its weight of  $NaCl$  and melted under 2 atmospheres' pressure.

The electrolyte analyzes the same as that of Example V and is used in the same way.

What is claimed is:

The method of producing coarsely crystalline zirconium free from  $ZrCl$  as a deposit adherent to the cathode which consists in making comminuted zirconium in an annular steel basket an anode in a cell having an inert cathode centrally located with respect to said anode and a molten electrolyte at about  $850^\circ C$ . consisting of sodium chloride in which is dissolved 2-6% zirconium as chloride, average valence 2.0-2.4 and sodium as determined by hydrogen evolution in acidified ferric salt solution 1-2.0%, passing a direct current through the cell at a cathode current density of about 500 amperes per sq. ft. and an anode current density of less than 1 ampere per sq. ft. and maintaining during the electrolysis a partial pressure of  $ZrCl_4$  of about 75 mm. of mercury.

#### References Cited in the file of this patent

#### UNITED STATES PATENTS

|           |               |               |
|-----------|---------------|---------------|
| 2,760,930 | Alpert et al. | Aug. 28, 1956 |
| 2,785,066 | Dean          | Mar. 12, 1957 |
| 2,834,727 | Gullett       | May 13, 1958  |

#### FOREIGN PATENTS

|           |        |               |
|-----------|--------|---------------|
| 1,126,457 | France | Nov. 23, 1956 |
|-----------|--------|---------------|